# EUROPEAN PATENT SPECIFICATION

(11) **EP 0 150 517 B1**
(45) Date of publication and mention of the grant of the patent: **23.12.1987**
(21) Application number: 84200099.4
(22) Date of filing: 26.01.1984
(51) Int. Cl.: G03C 1/37, G03C 5/26

(54) **Photographic elements and liquide for the processing of such elements containing a biocide**
Biocid enthaltende photographische Elemente und Lösungen,und deren Behandlung
Eléments photographiques et liquides contenant un biocide pour le traitement de ces éléments

(43) Date of publication of application: 07.08.1985
(73) Proprietor: AGFA-GEVAERT naamloze vennootschap, 2640 Mortsel (BE)
(72) Inventor: Kockelbergh, Godfried Antoon, B-2510 Mortsel (BE)

## Description

The present invention relates to photographic elements and liquids for the manufacture or processing of such elements containing a biocide.

In order to prevent the degradation of photographic elements containing a hydrophilic colloid, e.g. containing gelatin being an ideal nutrient for bacteria and fungi, it is necessary to add a biocide, usually phenol to kill these micro-organisms. Amongst the phenols used are phenol itself, thymol and p-chloro-m-cresol.

Phenols have a particularly unpleasant smell, are toxic for mammals, irritate the skin and have therefore to be manipulated with care. Moreover, they have a too small solubility in acidic aqueous media so that they may be incompatible with acidified photographic compositions e.g. particular silver halide gelatin coating compositions and acidic processing solutions from which the biocide could be applied by imbibition into the photographic element.

Phenols as biocide in photographic compositions cannot be replaced by any biocide suitable for industrial use since many of the known biocides affect the sensitometric properties of the photographic elements prepared or treated with compositions containing them.

In GB-A-1,177,048 nitro-alcohols have been described as useful compounds for inhibiting biological growth in acidic photographic processing compositions.

According to the present invention a photographic element containing a hydrophilic colloid and a biocide is provided, characterized in that said biocide is 5-bromo-5-nitro-1,3-dioxan having the following structural formula:

The synthesis of 5-bromo-5-nitro-1,3-dioxan and its use as a preservative for cosmetics is described in J. Soc. Cosmet. Chem., 28, 427-439 - August 1977.

In the photographic element the growth of both fungi and bacteria is inhibited without disadvantageously affecting the sensitometric properties of said element.

Said dioxan is active against gram-positive and gram-negative bacteria as well as fungi in concentrations otO.02 to 0.05% by weight in aqueous solutions and solid hydrophilic colloid compositions. Toxicological and dermatological investigations have demonstrated that said dioxan is tolerated by mammals without adverse reactions.

The 5-bromo-5-nitro-1,3-dioxan is soluble in neutral, alkaline as well as acidic aqueous media and is compatible (without affecting transparency) with layers containing a proteinaceous colloid binder such as gelatin.

Photographic materials containing according to the present invention a dioxan-biocide in a hydrophilic colloid medium are, e.g. photographic elements containing (a) silver halide hydrophilic colloid emulsion layer(s) and elements that are not photosensitive but contain a hydrophilic colloid layer and are suited for use as image-receiving element in conjunction with a photographic silver halide element in a diffusion transfer reversal (DTR-) processing.

The optimum amount of the said dioxan biocide in elements for photographic image formation, coating compositions and processing liquids is readily determined by comparing the growth of bacteria and fungi with control liquids (solutions, emulsions or suspensions) and solid hydrophilic colloid media containing no biocide and those containing increasing concentrations thereof.

Photographic elements, e.g. silver halide emulsion layer materials, containing in one or more hydrophilic colloid layers a coverage of 2 milligram to 30 milligram per m² of the 5-bromo-5-nitro-1,3-dioxan are adequately protected against microbiological growth.

The bactericidal activity of 5-bromo-5-nitro-1,3-dioxan has been found to be at least 20 times as strong as that of phenol. The fungicidal activity compared with that of phenol is still higher. From comparative tests could further be concluded that 5-bromo-5-nitro-1,3-dioxan is a stronger bactericide than the nitro-propanols described in the already mentioned GB-A-1,177,048, which nitro-propanols are only stable in acidic medium.

The said dioxan-biocide can be incorporated into the coating composition of a silver halide emulsion layer or other colloid layers in water-permeable relationship therewith according to any technique known by those skilled in the art for incorporating photographic ingredients, such as colour couplers, into colloid compositions.

A survey of techniques suitable for incorporating photographic ingredients into photographic elements has been given in GB-P 1,546,371. For example, they are incorporated from solutions in organic water-miscible solvents.

The dioxan-biocide can be incorporated in solutions or dispersions of photographic ingredients that include e.g. aqueous dispersions of polymers (latices) applied in the production of photographic elements. Since these dispersions or solutions are normally stored for days or weeks before being incorporated in the coating composition of a layer of a photographic element the dioxan-biocide also exerts its favourable bactericide activity on these solutions or dispersions.

A liquid coating composition used in the manufacture of the present photographic material contains, e.g., said dioxan-biocide in a concentration in the range of 50 milligram to 500 milligram per litre.

According to a particular embodiment the hydrophilic colloid(s) serving as binding agent(s) are used in admixture with a synthetic polymer applied from a latex as described e.g. in EP-A-0010335 and GB-P 1,453,057, and such mixture contains the said dioxan-biocide already before use in the preparation of an element for photographic image formation according to the present invention.

The said dioxan-biocide can be used in conjunction with any kind of photographic silver halide emulsion where the silver salts can be, e.g., silver bromide, silver iodide, silver chloride or mixed silver halides such as silver chlorobromide, silver bromoiodide, and silver chlorobromoiodide. In these silver halide emulsions the latent images may be formed predominantly at the surface of the silver halide crystals of formed predominantly inside the silver halide crystals.

The hydrophilic colloid used as the vehicle for the silver halide can be, e.g., gelatin, colloidal albumin, zein, casein, a cellulose derivative, e.g. carboxymethylcellulose, a synthetic hydrophilic colloid such as polyvinyl alcohol or poly-N-vinylpyrrolidone. If desired, compatible mixtures of two or more of these colloids can be employed for dispersing the silver halide.

Light-sensitive silver halide emulsions used in the preparation of a photographic element according to the present invention can be sensitized chemically as well as optically. They can be sensitized chemically by carrying out the ripening in the presence of small amounts of sulphur-containing compounds such as allylthiocyanate, allyl thiourea, or sodium thiosulphate. The emulsions can also be sensitized by means of reducing agents, e.g., tin compounds as described in FR-A-1,146,955 and in BE-A-568,687, imino- aminomethane salphinic acid compounds as described in GB-A-789,823 and small amounts of noble metal compounds such as gold, platinum, palladium, iridium, ruthenium, and rhodium compounds. They can be sensitized optically by means of cyanine and merocyanine dyes.

The said silver halide emulsions can also comprise compounds that sensitize the emulsions by development acceleration e.g. compounds of the polyoxyalkylene type such as alkylene oxide condensation products as described i.a. in USA2,531,832 2,533,990, in GB-A-920,637 - 940,051 - 945,340 - 991,608 and 1,091,705; onium derivatives of amino-N-oxides as described in GB-A-1,121,696, and thioether compounds as described, e.g., in GB-A-1,455,413 and 1,528,951.

The silver halide emulsions may be of the black-and-white or colour type, so that they may contain any type of colour coupler, dye or dye precursor, e.g. as is used in common silver halide colour photography or dye diffusion transfer photography.

The dioxan-biocide can be used in black-and-white and colour materials for the positive-negative photography or the reversal photography.

Further, the emulsions may comprise stabilizers e.g. heterocyclic nitrogen-containing thioxo compounds such as benzothiazoline-2-thione and 1-phenyl-2-tetrazoline-5-thione and compounds of the hydroxytriazolpyrimidine type. They can also be stabilized with mercury compounds such as the mercury compounds described in BE-A-524,121 and 677,337, and in GB-A-1,173,609.

The light-sensitive silver halide emulsions or hydrophilic colloid layers containing said dioxan-biocide may also comprise any other kind of ingredient such as those described therefor in Research Disclosure no. 17,643 of December 1978.

The silver halide emulsions containing said dioxan-biocide can be coated onto a wide variety of supports. Typical supports are e.g. cellulose ester film, polyvinylacetal film, polystyrene film, polyethylene terephthalate film and related films or resinous materials as well as glass, paper, or paper boards, such as paper or paper board coated with plastics, e.g. polyethylene-coated paper.

According to an embodiment of the invention the 5-bromo-5-nitro-1,3-dioxan is used in a silver halide developing solution, silver halide complexing solution or a silver metal bleaching solution.

When incorporated in a treating solution for a photographic silver halide material the dioxan-biocide is used e.g. in a concentration of 50 milligram to 500 milligram per litre.

Such treating solution is, e.g., a silver halide developing solution, silver halide complexing solution or silver metal bleaching solution.

The following comparative test example illustrates the present invention.

### Comparative example

The inhibition of biological growth with phenol, 2-hydroxymethyl-2-nitro-1,3-propanediol, 2-bromo-2-nitro-1,3-propanediol and 5-bromo-5-nitro-1,3-dioxan respectively was compared at various concentrations in a 6% by weight aqueous solution of gelatin.

One group of the test solutions was infected in a same concentration by bacteria isolated from a spoiled gelatin solution and another group of test solutions was infected by fungi likewise isolated from a spoiled gelatin solution.

The infected test solutions were kept at 37°C to promote biological growth and samples of 1 ml were taken thereof after 24 h and 3 weeks.

The 1 ml samples were used to infect commercial nutrients for bacteria and fungi respectively which were incubated under the same circumstances for the development of colonies of micro-organisms.

The following table contains a survey of the results obtained. Herein (-) stands for the absence of microbiological growth, and (+) for a considerable microbiological growth.

## Claims

1. A photographic element containing a hydrophilic colloid and a biocide, characterized in that the biocide is 5-bromo-5-nitro-1,3-dioxan having the following structural formula:

2. Photographic element according to claim 1, characterized in that said element contains (a) silver halide emulsion layer(s).

3. Photographic element according to claim 1 or 2, characterized in that said element contains said biocide at a coverage of 2 milligram to 30 milligram per m².

4. Liquid for treating a photographic element which liquid is a silver halide developing solution, silver halide complexing solution or a silver metal bleaching solution containing a biocide, characterized in that the biocide corresponds to the following formula:

5. Liquid for treating a photographic element according to claim 4, characterized in that said liquid contains said biocide in a concentration in the range of 50 milligram to 500 milligram per litre.

## Patentansprüche

1. Photographisches Element, das ein hydrophiles Kolloid und ein Schädlingbekämpfungsmittel enthält, dadurch gekennzeichnet, daß letzteres 5-Brom-5-nitro-1,3-dioxan entsprechend der folgenden Strukturformel ist:

2. Photographisches Element nach Anspruch 1, dadurch gekennzeichnet, daß es eine oder mehrere Silberhalogenidemulsionsschichten enthält.

3. Photographisches Element nach Anspruch 1, dadurch gekennzeichnet, daß es das Schädlingbekämpfungsmittel in einem Verhältnis von 2-30 mg pro m² enthält.

4. Flüssigkeit zum Behandeln eines photographischen Elementes, welche eine Silberhalogenid-Entwicklerlösung, eine Silberhalogenid komplexierende Lösung oder eine Silbermetall ausbleichende Lösung ist, die ein Schädlingbekämpfungsmittel enthält, dadurch gekennzeichnet, daß das Schädlingbekämpfungsmittel der folgenden Formel entspricht:

5. Flüssigkeit zum Behandeln eines photographischen Elementes nach Anspruch 4, dadurch gekennzeichnet, daß sie das Schädlingbekämpfungsmittel in einer Konzentration von 50-500 mg pro Liter enthält.

## Revendications

1. Elément photographique contenant un colloîde hydrophile et un biocide, caractérisé en ce que ce biocide est le 5-bromo-5-nitrol-1,3-dioxanne répondant à la formule structurale suivante:

2. Elément photographique selon la revendication 1, caractérisé en ce qu'il contient une ou plusieurs couches d'émulsions aux halogénures d'argent.

3. Elément photographique selon la revendication 1 ou 2, caractérisé en ce qu'il contient ce biocide à raison de 2 mg à 30 mg/m².

4. Liquide pour le traitement d'un élément photographique, ce liquide étant une solution dévelop- patrice pour les halogénures d'argent, une solution complexant les halogénures d'argent ou une solution de blanchiment de l'argent métallique contenant un biocide, caractérisé en ce que le biocide répond à la formule suivante:

5. Liquide pour le traitement d'un élément photographique selon la revendication 4, caractérisé en ce qu'il contient ce biocide en une concentration se situant dans l'intervalle allant de 50 mg à 500 mg/litre.
